

## UNITED STATES PATENT OFFICE

GEORGE HOLLAND ELLIS, OF SONDON, NEAR DERBY, ENGLAND, ASSIGNOR TO  
CELANESE CORPORATION OF AMERICA, A CORPORATION OF DELAWARE

## TREATMENT OF CELLULOSE DERIVATIVES

No Drawing. Application filed September 7, 1926, Serial No. 134,138, and in Great Britain April 10, 1926.

This invention relates to the dyeing, printing or stencilling of artificial yarns, threads, filaments, fabrics, films or other products made of or containing cellulose acetate.

5 I have now found that particularly useful and desirable results may be obtained by the employment of a solubilizing agent or agents consisting of or comprising a sulpho-aromatic ricinoleic acid or a salt thereof, that is 50 to say a body which is capable of being obtained by the treatment of a mixture of castor oil and an aromatic compound, for example benzene, phenol or naphthalene, with sulphuric acid; or a salt of such a body, for instance the alkali or ammonium salt.

Accordingly the present invention consists in the dyeing, printing, or stencilling of cellulose acetate or goods containing the same with any insoluble or relatively insoluble colouring 55 matters or organic compounds having affinity for cellulose acetate or capable of colouring the same, in the form of soluble or more soluble modifications prepared by treatment with solubilizing agents consisting of 60 or comprising one or more bodies being sulpho-aromatic ricinoleic acids, for example sulpho-benzene ricinoleic acid, sulpho-phenol ricinoleic acid, or sulpho-naphthalene ricinoleic acid; or salts of such bodies, for instance the alkali or ammonium salts of such 65 bodies.

The dyebaths for applying the colouring matters or compounds solubilized according to the present invention may be acid, neutral, 70 or alkaline and it is also found that good results may be obtained even if hard water be employed in making up the dyebath.

Any insoluble or relatively insoluble colouring matter or compound having affinity 75 for cellulose acetate may be employed and the following may be instanced, though it is to be understood that such examples are not intended to limit the invention, which contemplates as stated above the employment of 80 any insoluble or relatively insoluble colour-

ing matter or compound having the requisite affinity. Thus I may employ the colouring matters or organic compounds more particularly referred to in my previous British specification No. 219349, and U. S. Patent No.

1,618,413, for instance non-sulphonated or other insoluble or relatively insoluble derivatives of the "azo" class, simple or amino bases (e. g. para nitraniline, meta nitraniline, benzidine, dianisidine, dimethyl aniline, alpha naphthylamine or diphenylamine) for application for dyeing or colouring the cellulose acetate by the azoic or development process, unreduced indophenols (aryl or substituted aryl benzo- or naphthaquinone monoimides), or insoluble or relatively insoluble colouring matters of the following classes:

Polyaryl methane, oxazine, azine, thiazine, unreduced indigoid or basic derivatives of the anthraquinone series; insoluble or relatively insoluble pyrazolone derivatives e. g. unsulphonated azo derivatives of pyrazolone compounds, such as are referred to in my previous British specification No. 224681 and in my U. S. Patent No. 1,600,277; unreduced 70 vat dyestuffs of the anthraquinone series as referred to in my previous British specification No. 227183 and in my U. S. Patent No. 1,641,965, for instance those marketed under the registered trade marks Indanthrene, 75 Cibanone, Algol and Helindone; insoluble or relatively insoluble nitroderivatives of diarylamines such as those referred to in my previous British specification No. 237943 and in my U. S. Patent No. 1,618,415; insoluble 80 or relatively insoluble acidyl derivatives of aminoanthraquinones or of substituted aminoanthraquinones, containing one or more aliphatic acidylamino groups, such as those referred to in my application for British Patent No. 26576 of 1925 and my U. S. application S. No. 98,614 of 30 March 1926; insoluble or relatively insoluble colouring matters or compounds of the stilbene group containing no sulpho groups in their constitution,

85 90

such as those referred to in my application for British Patent No. 7317 of 1925 and in my U. S. application S. No. 93,779 of 10th March 1926.

5 The colouring matters or compounds for use in the present invention will usually contain no strongly acidic groups such as the sulpho group, and when basic colouring matters or compounds are employed they are alter-  
10 ways used in the form of the base and not in the form of salts such as the hydrochloride.

The solubilization may be effected by mixing or grinding the insoluble or relatively insoluble colouring matters or compounds with 15 one or more of the solubilizing agents of the present invention, in presence or absence of water,—if desired in presence of comparatively large quantities of water with subsequent concentration,—and heating if necessary, the solubilized modifications being filtered if required before addition to the dye-baths or other preparations for dyeing or otherwise colouring the goods. The dyeing, printing or stencilling may be effected in the 20 usual manner.

If the colouring matter or compound contains diazotizable amino groups, it may be diazotized and developed on the material to form a further dyestuff or dyestuffs.

25 30 When dyeings or colourings are to be produced by the azoic process the insoluble or relatively insoluble component (whether base or developer or both) may be solubilized with the agents of the present invention and the dyeing and developing conducted as usual.

Other colouring matters which are not deleteriously affected by the solubilizing agents of the present invention may if desired, be dyed on the material together with the colouring matters or compounds treated according to the present invention.

Mixed goods may be dyed or otherwise coloured in uniform or contrasting effects with 45 or without employment of other dyestuffs or components according to the character of the nonacetate portion of the goods, said other dyestuffs being applied before, after, or, if not deleteriously affected thereby, together 50 with the insoluble dyestuffs or compounds treated according to the present invention.

The solubilizing agents of the present invention may be prepared in any known or suitable way. The following Example A illustrates one convenient method of preparing them.

Example A.—Method of preparing the solubilizing agent.  
172 lbs. of sulphuric acid (monohydrate) 60 are charged into a jacketed mixer, 60 lbs. of naphthalene added, and 60 lbs. of castor oil run in during one hour, cooling water being run through the jacket so that the temperature rises only to 25–30° C.

65 The water is then run off from the jacket,

and steam turned on very slightly, the rate of heating being regulated by the amount of frothing of the mixture. Usually it is possible to raise the temperature to 95–100° C. in 8 hours, when most of the frothing will have ceased. The temperature is now raised to 105° C. and kept at this degree for 2½ hours, after which it is allowed to cool to a moderate temperature. It is now blown into 70 130 gallons of 20% brine, stirred well and allowed to settle. The brine is now drawn off and the layer of oil given two further similar treatments, after which the separated oil is mixed with 20–30 lbs. of hot water, neutralized with 30% caustic soda solution, and finally made up to 312 lbs. by addition of water.

75 The following are some examples of the manner in which the invention may be performed it being understood that these are given only by way of illustration and can be varied widely without departing from the invention.

80 Example 1.—To dye 100 lbs. of cellulose acetate yarn in hank form a bright golden yellow colour:—

85 1 lb. of 4' hydroxy 2:4 dinitrodiphenylamine is ground in a suitable apparatus with 3 lbs. of sulpho-naphthalene ricinoleic acid, sodium salt, prepared as in Example A, and water added to make to 10 lbs.

90 The paste thus obtained is treated with 10 gallons of boiling water and added to a dye-bath containing 300 gallons of soft water in which have been dissolved three pounds of olive oil soap. The well scoured yarn is now entered and the temperature of the bath raised during ¾ of an hour to 75° C. and maintained at this temperature a further ¾ of an hour. The yarn, which is now dyed 100 a full golden yellow colour is washed off in soft water, and may be dried or otherwise treated as desired.

95 Example 2.—To dye 100 lbs. of cellulose acetate yarn in hank form a full yellow shade:—

100 1 lb. of alpha acetyl amino anthraquinone is ground to a fine powder, and added to 4 lbs. of neutral sodium sulpho naphthalene ricinoleate prepared as in Example A. The whole is now heated to 75–80° C. with stirring till as homogeneous as possible, diluted to 10 gallons with boiling water, and added to the dyebath containing 300 gallons of ordinary tap water. The goods are now entered, the temperature raised to 75–80° C. in ¾ of an hour and maintained at this degree for ¾ of an hour. The goods, which are now dyed a full greenish yellow are washed off and may be dried or otherwise 110 treated as desired.

115 Example 3.—To dye 100 lbs. of cellulose acetate yarn in hank form a pure blue shade:—

120 1½ lbs. of the indophenol obtained by oxi- 125

dizing p. amino diethylaniline and alpha naphthol in alkaline solution (1: p. diethylamino phenyl 4: naphthoquinone monoimide) are reduced to a fine state of division and stirred at a moderate temperature into 5 lbs. of neutral sodium sulpho naphthalene ricinoleate prepared as in Example A. When as homogeneous as possible the dispersion is diluted with 10 gallons of warm water and 10 poured through a filter cloth into a dyebath containing 300 gallons of water. The goods are now entered and dyeing is carried out as in Examples 1 and 2. The goods which are dyed a full pure blue shade, are well washed off and may now be dried or otherwise treated as desired.

*Example 4.*—To dye 100 lbs. of wool-cellulose acetate mixed goods in hank forms:—

Cellulose acetate, yellow.

20 Wool, red.

Ratio wool-cellulose acetate:—2:1.

25  $\frac{1}{4}$  lb. of anilineazo-1:phenyl-3:methyl-5:pyrazolone is dispersed in 2 lbs. of sodium sulpho naphthalene ricinoleate (prepared as in Example A) by grinding or other suitable means, diluted to 5 gallons with boiling water, and added to a 300 gallon dyebath in which has previously been dissolved 1½ lbs. of Azo Rhodine 2G. (Colour index No. 31). 30 The scoured goods are now entered and the temperature raised gradually, during ¾ of an hour to 70–75° C. and maintained for a further ¾ of an hour. Exhaustion is assisted by the addition of 3 lbs. of acetic acid during ¼ of an hour intervals at 70–75° C. The goods which are now dyed the requisite shades are washed off well, and may now be dried or otherwise treated as desired.

40 *Example 5.*—To dye a full bluish black on 100 lbs. of cellulose acetate yarn in hank form:—

45 2 lbs. of benzene azo alpha naphthylamine are dispersed in 8 lbs. of sodium sulpho naphthalene ricinoleate prepared as in Example A, and applied to the cellulose acetate yarn by the methods illustrated in Examples 1 and 2. The goods which are dyed a full golden shade, are well washed off and are now 50 ready for the diazotization bath.

#### Diazotization

55 5 lbs. of sodium nitrite are dissolved in a bath containing 150 gallons of water at 5–10° C. 20 lbs. of 30% hydrochloric acid, suitably diluted, are now added, the bath well stirred and the goods entered immediately. Diazotization is complete in half an hour, and the goods are lifted, well washed off in cold water 60 and entered immediately into the coupling bath.

#### Coupling bath

65 4 lbs. of beta oxynaphthoic acid are dissolved in water containing 1 lb. of caustic soda, 20 lbs. of sodium sulpho naphthalene

ricinoleic acid prepared as in Example A are now added, and the whole stirred well. The bath, which is at 15–20° C. is now rendered faintly acid to litmus paper by careful addition of a 10% solution of formic acid, and the goods from the previous treatment entered. 70 Coupling is carried out cold for ¾ of an hour and the temperature then slowly raised to 60° C. being maintained a further ¼ of an hour at this temperature.

The goods are now lifted, rinsed, soaped for 10 minutes in a ¼% soap solution at 45° C. and well washed off.

75 They are dyed a full bloomy black and may now be dried or otherwise treated as desired.

80 The term dyeing in the appended claims is intended to include printing and stencilling, while the term "relatively water-insoluble organic compounds capable of colouring cellulose acetate" is to be understood to include any insoluble or relatively insoluble colouring matter or organic compound having affinity for cellulose acetate or capable of colouring the same or any component (base or developer) capable of application by the azoic or development process.

85 What I claim and desire to secure by Letters Patent is:—

90 1. Process for dyeing materials comprising cellulose acetate, comprising applying thereto aqueous dispersions of relatively water-insoluble organic compounds capable of coloring cellulose acetate prepared by pre-treating the compounds with a solubilizing agent comprising a compound selected from the group consisting of sulpho-aromatic ricinoleic acids and their soluble salts.

95 2. Process for dyeing materials comprising cellulose acetate, comprising applying thereto aqueous dispersions of relatively water-insoluble organic compounds capable of coloring cellulose acetate prepared by pre-treating the compounds with a solubilizing agent comprising a soluble salt of a sulpho-aromatic ricinoleic acid.

100 105 3. Process for dyeing materials comprising cellulose acetate, comprising applying thereto aqueous dispersions of relatively water-insoluble organic compounds capable of coloring cellulose acetate, prepared by pre-treating the compounds with a solubilizing agent comprising a sodium salt of a sulpho-aromatic ricinoleic acid.

110 115 4. Process for dyeing materials comprising cellulose acetate, comprising applying thereto aqueous dispersions of relatively water-insoluble organic compounds capable of coloring cellulose acetate prepared by pre-treating the compounds with a solubilizing agent comprising a compound selected from the group consisting of sulpho-naphthalene ricinoleic acids and their soluble salts.

120 125 5. Process for dyeing materials comprising cellulose acetate, comprising applying

130

135

140

145

150

155

160

165

170

175

180

185

- thereto aqueous dispersions of relatively water-insoluble organic compounds capable of coloring cellulose acetate prepared by pretreating the compounds with a solubilizing agent comprising a soluble salt of a sulpho-naphthalene ricinoleic acid. 70
6. Process for dyeing materials comprising cellulose acetate, comprising applying thereto aqueous dispersions of relatively water-insoluble organic compounds capable of coloring cellulose acetate prepared by pretreating the compounds with a solubilizing agent comprising a sodium salt of a sulpho-naphthalene ricinoleic acid. 75
15. 7. Process for dyeing materials comprising cellulose acetate, comprising applying thereto aqueous dispersions of relatively water-insoluble amino compounds prepared by pretreating the compounds with a solubilizing agent comprising a compound selected from the group consisting of sulpho-aromatic ricinoleic acids and their soluble salts and thereafter diazotizing and developing on the material. 80
20. 8. Dyeing preparations comprising relatively water-insoluble organic compounds pretreated with a solubilizing agent comprising a compound selected from the group consisting of sulpho-aromatic ricinoleic acids and their soluble salts. 85
25. 9. Dyeing preparations comprising relatively water-insoluble organic compounds pretreated with a solubilizing agent comprising a soluble salt of a sulpho-aromatic ricinoleic acid. 90
30. 10. Dyeing preparations comprising relatively water-insoluble organic compounds pretreated with a solubilizing agent comprising a soluble salt of a compound selected from the group consisting of sulpho-naphthalene ricinoleic acids and their soluble salts. 95
35. 11. Dyeing preparations comprising relatively water-insoluble organic compounds pretreated with a solubilizing agent comprising a sulpho-naphthalene ricinoleic acid. 100
40. 12. Process for dyeing materials comprising cellulose acetate, comprising applying thereto aqueous dispersions of relatively water-insoluble organic compounds capable of coloring cellulose acetate prepared by pretreating the compounds with a solubilizing agent comprising a compound selected from the group consisting of sulpho-benzene ricinoleic acids and their soluble salts. 105
45. 13. Process for dyeing materials comprising cellulose acetate, comprising applying thereto aqueous dispersions of relatively water-insoluble organic compounds capable of coloring cellulose acetate prepared by pretreating the compounds with a solubilizing agent comprising a compound selected from the group consisting of sulpho-phenol ricinoleic acids and their soluble salts. 110
50. 14. Dyeing preparations comprising relatively water-insoluble organic compounds pretreated with a solubilizing agent comprising a compound selected from the group consisting of sulpho-benzene ricinoleic acids and their soluble salts. 115
55. 15. Dyeing preparations comprising relatively water-insoluble organic compounds pretreated with a solubilizing agent comprising a compound selected from the group consisting of sulpho-phenol ricinoleic acids and their soluble salts. 120
60. 16. Dyeing preparations comprising relatively water-insoluble organic compounds pretreated with a solubilizing agent comprising a compound selected from the group consisting of sulpho-phenol ricinoleic acids and their soluble salts. 125
65. 17. Dyeing preparations comprising relatively water-insoluble organic compounds pretreated with a solubilizing agent comprising a compound selected from the group consisting of sulpho-phenol ricinoleic acids and their soluble salts. 130

In testimony whereof I have hereunto subscribed my name.

GEORGE HOLLAND ELLIS.